

3,250,711  
**GEAR LUBRICANT**  
Curtis L. Early, Alton, Ill., assignor to Shell Oil Company,  
New York, N.Y., a corporation of Delaware  
No Drawing. Filed Mar. 6, 1964, Ser. No. 350,103  
3 Claims. (Cl. 252—37.2)

This invention relates to improved gear oils comprising a blend of two selected petroleum stocks as the base for the extreme pressure gear oil additive mixture of the present invention, which functions synergistically.

It is well known in the lubricant art that one of the most effective and economical additive combinations for use in gear oils is a mixture of lead naphthenate and a sulfurized fatty oil. Gear oils containing this additive mixture have been used successfully for years in commercial applications such as steel mills, power generating plants, etc. However, current operating conditions have become progressively more severe due to heavier unit gear loading, higher bulk oil operating temperatures, etc. This results in rapid oxidation of the oil, sludging, coprecipitation and depletion of the additives mentioned above and general breakdown of the lubricant resulting in severe damage to equipment, increase in repair costs, and loss in time and production.

It has now been discovered that an oil blend consisting of a mixture of 55–85% of a particular high viscosity index bright stock fraction and 45–15% of a high viscosity index mineral lubricating oil, both fractions having a viscosity index of at least 80, preferably 90–140 and both fractions being rich in aromatics, function not only as an excellent base vehicle of the conventional gear oil additive mixture mentioned, namely a mixture of lead naphthenate and a sulfurized fatty oil or derivative thereof such as sulfurized sperm oil, but the base oil blend acts synergistically to activate the extreme pressure life of gear oil additive mixture so that it is increased many fold, namely from 1 to 10 times that of commercial gear oils containing lead naphthenate and sulfurized fatty products, and inhibits additive depletion and oxidation of the composition. The manner in which the oil blend of the present invention functions in the manner described is not understood, except for the fact that in order to produce the desired results, the base oil blend must be carefully selected and blended in specific proportions, each fraction of which must possess the following properties: (1) the bright stock fraction must be rich in aromatics (5–70%) and have a viscosity index of at least 80, preferably between 90 and 110 and is obtained during the refining of mineral oils from the short residue after the distillate fractions have been removed. The short residue is dewaxed and deasphalted and if desired solvent and clay-treated. The raffinate which remains after this treatment is called bright stock.

The bright stocks should have the following range of properties:

TABLE I.—PROPERTIES OF BRIGHT STOCKS

|                         |                                                   |
|-------------------------|---------------------------------------------------|
| Viscosity, SUS,         |                                                   |
| 100° F. ....            | >1250, usually 1250–11,000, preferably 1500–3500. |
| Viscosity, SUS,         |                                                   |
| 210° F. ....            | >75, usually 125–325, preferably 150–250.         |
| Viscosity index ....    | >+80, preferably +85–110.                         |
| Aniline point ....      | >100, preferably >115.                            |
| Flash, ° F. ....        | >475, preferably >500.                            |
| Fire, ° F. ....         | >550, preferably >600.                            |
| Pour point, ° F. ....   | +25 maximum, preferably lower than +15°.          |
| Percent aromatics ....  | >15.                                              |
| Percent naphthenes .... | <35.                                              |
| Percent paraffins ....  | At least 60.                                      |

TABLE II.—EXAMPLES OF TYPICAL BRIGHT STOCKS

|    |                                        | Mid-Continent bright stock |                  | Pennsyl-vania bright stock |
|----|----------------------------------------|----------------------------|------------------|----------------------------|
|    |                                        | Mild extraction            | Heavy extraction |                            |
| 10 | Viscosity, SUS, 100° F. ....           | 2,569                      | 2,049            | 2,109                      |
|    | Viscosity, SUS, 210° F. ....           | 141                        | 131              | 144                        |
|    | Viscosity index ....                   | 85                         | 93               | 102                        |
| 15 | Ring analysis:                         |                            |                  |                            |
|    | Aromatic. ....                         | 9                          | 5                | 5                          |
|    | Naphthenes. ....                       | 19                         | 19               | 16                         |
|    | Paraffins. ....                        | 72                         | 76               | 79                         |
|    | Ratio of paraffins to naphthenes. .... | 3.8                        | 3.62             | 4.95                       |
|    | Average mol weight. ....               | 685                        | 675              | 730                        |
|    | Average rings per mol. ....            | 3.4                        | 2.9              | 3.0                        |

TABLE III.—SPECIFICATIONS FOR TYPICAL MID-CONTINENT BRIGHT STOCKS

|    |                                 | Unfiltered | Filtered   |
|----|---------------------------------|------------|------------|
| 20 | Gravity, ° API, minimum. ....   | 25.5       | 24.5       |
|    | Color, NPA. ....                | 8+         | Dark green |
|    | Pour point, ° F., maximum. .... | 10         | 10         |
|    | Flash, ° F., minimum. ....      | 540        | 580        |
|    | Fire, ° F., minimum. ....       | 615        | 655        |
| 25 | Viscosity, SUS, 210° F. ....    | 150–170    | 200–215    |
|    | Viscosity index, minimum. ....  | 90         | 90         |

The other portion of the oil blend is a high viscosity index lubricating oil distillate fraction and specifically is a refined distillate fraction having a viscosity index of at least 90, preferably 90–110, an SUS viscosity at 100° F. in the range of 100–600, and containing substantial proportions of heterocyclic aromatics such as sulfur-containing aromatics (2–10%) such as benzothiophenes, dibenzothiophenes, thiophenacenaphthylenes, thiophenophenanthrenes, thiophenopyrenes, etc. Such a typical petroleum fraction will be referred to as fraction (Y) and such a fraction derived from an East Texas Crude has the following properties:

30 Viscosity, SUS, at 100° F. .... 250  
Viscosity index .... 90–95  
Analysis (incremental ultraviolet absorption):  
40 Monoaromatics, percent .... 14  
Polyaromatics, of which 13–17% are diaromatics containing thiophenic structures, e.g., benzo- and dibenzothiophenes, percent .... 21  
45 Polar-containing resins, percent .... 3  
Essentially balance—saturates.

50 Base blends which are particularly preferred are:  
(A)

60% Bright stock (unfiltered—Table III)  
40% HVI oil fraction (Y)

(B)

70% Bright stock (12% aromatics)  
30% HVI oil fraction (Y)

60 The additive combination which is synergistically activated, stabilized and its depletion inhibited by the base blend described comprises of a mixture of 1–10% (preferably 2–5%) lead naphthenate and 1–10% (preferably 3–6%) by weight of sulfurized long-chain fatty oil product such as sulfurized sperm oil.

65 The lead naphthenate utilized in the lubricant can be prepared from naphthenic acids obtained in the refining of petroleum, particularly the naphthenic acids derived from lubricating oil fractions. Moreover, the naphthenic acids can contain some non-saponifiable mineral oil which may vary up to 30% or more. A typical lead naphthenate, prepared from lubricating oil naphthenic acids having a

non-saponifiable content of about 23%, has a PbO content of roughly about 20% by weight. Lead naphthenate prepared from naphthenic acids essentially freed from non-saponifiable content will run about 30% PbO content.

The sulfurized fatty material containing 10-40% sulfur in the molecule can be sulfurized sperm oil (20-30% S). A sulfurized sperm oil of this type is available from Carlisle Chemical Works as Base 100-S or 120-S, the latter of which has the following properties:

|                               |                                                       |    |
|-------------------------------|-------------------------------------------------------|----|
| Sulfur                        | 13.0 percent.                                         | 10 |
| Sperm oil                     | 87.0 percent.                                         |    |
| API gravity at 60° F.         | 14.8.                                                 | 5  |
| Lbs./gal. at 60° F.           | 8.05.                                                 |    |
| Pour point, ASTM              | 65° F.                                                | 15 |
| Flash point, COC              | 445° F.                                               |    |
| Fire point, COC               | 495° F.                                               |    |
| Unsaponifiable, AOCS          | 35 percent.                                           | 20 |
| Viscosity at 210° F., SSU     | 250.                                                  |    |
| Corrosion, ASTM               | Positive.                                             |    |
| Color, ASTM (2 1/4% solution) | 4.                                                    |    |
| Solubility                    | Completely soluble in practically all petroleum oils. |    |

#### Sulfur separation

In addition to the two essential additives, a minor amount (1-5% by weight) of a secondary additive can be incorporated such as a polyolefinic thickener, e.g., polybutene, polyisobutylene, alkylated naphthalene, or a foam inhibitor, e.g., dimethyl silicone polymers having a viscosity in centistokes at 25° C. of from 100 to 1000, preferably between 200 and 300; antioxidants such as alkyl phenols and bisphenols, e.g., di- and trialkylphenols, for instance 2,4-, 2,3-, 3,4-, 2,6- and 3,5-diamyl phenol, 2,4-dimethyl-6-tertbutyl phenol, 2,6-diterbtbutyl-4-methylphenol; bisphenols, e.g. 4,4'-methylene (2,6-diterbtbutyl phenol), 4,4'-thio bis (2,6-diterbtbutyl phenol); arylamines such as phenyl-alpha-naphthylamine or phenyl-beta-naphthylamine.

The following examples illustrate the invention:

- (I) Base blend (A):
  - +2.7% lead naphthenate
  - +4.0% sulfurized sperm oil (13% S)
  - +1% polyisobutylene (MW 1200)
  - +5 p.p.m. dimethyl silicone polymer (200 cs. at 25° C.)
- (II) Base blend (B):
  - +2.7% lead naphthenate
  - +4.0% sulfurized sperm oil (13% S)
  - +1% polyisobutylene (MW 1200)
  - +5 p.p.m. dimethyl silicone polymer (200 cs. at 25° C.)

- (III) Base blend (A):
  - +3.0% lead naphthenate
  - +4.5 sulfurized sperm oil
- (IV) Base blend (C):
  - 65% Bright stock (40% aromatics)
  - 35% HVI mineral lubricating oil (VI=90, Aromatics 35%)
  - +4% lead naphthenate
  - +4% sulfurized sperm oil
- (V) Base blend (D):
  - 65% Bright stock (30% aromatics)
  - 35% HVI mineral lubricating oil (VI=90, Aromatics 30%)
  - +2.5% lead naphthenate
  - +4% sulfurized sperm oil
- (VI) Base blend (A):
  - +2.7% lead naphthenate
  - +4.0% sulfurized sperm oil (13% S)
  - +1% polyisobutylene (MW 1200)
  - +1% polyisobutylene (MW 800)
  - +5 p.p.m. dimethyl silicone polymer (200 cs. at 25° C.)

The following compositions were subjected to the following tests and the results are shown in Table IV.

#### Tests

##### Oxidation Tests (X) 300° F. Bench Oxidation Test (BO Test).

In this method 300 ml. of test oil are oxidized in a cylindrical Pyrex glass cell at 300° F. with 5 liters air per hour for 168 hours. No catalyst is used.

The relative oxidation resistance of an oil is evaluated by viscosity increase and sludge formation during the test.

##### Oxidation Test (XX) Modified Turbine Oil Stability Test.

This test is a modification of ASTM Method D-943, "Oxidation Characteristics of Inhibited Steam Turbine Oils." In modifying ASTM D-943 for assessing the oxidation characteristics of Macoma blends, the test temperature is increased from 205° F. to 250° F., air instead of oxygen is used, water is omitted, and oil test life constitutes the number of hours of oxidation required to

double the original S.S.U. viscosity at 210° F.

Extreme Pressure Test: (XXX) Timken EP Test (Fed. Stand. method 6505-T).

##### Corrosion Test: (XXXX) Copper Strip Corrosion Test (ASTM-D-130).

The Copper Strip Corrosion Test, ASTM D-130, was used to evaluate the copper corrosivity at 212° F. This test was modified to evaluate also corrosivity of blends toward both copper and steel (AISI 1020) at 300° F. The appearance of metal panels after 3 hours' immersion at the required test temperature is used as an indication of the corrosive propensity of test oils.

TABLE IV

| Compositions                                                                                                               | (X)                            |                       |                 | Mg sludge per 10 g. | Max. lbs. passed | Cu cor. at 212° F. and 300° F. |
|----------------------------------------------------------------------------------------------------------------------------|--------------------------------|-----------------------|-----------------|---------------------|------------------|--------------------------------|
|                                                                                                                            | Percent S.S.U. at 210° F. inc. | Mg sludge at end test | Percent Pb loss |                     |                  |                                |
| (I)                                                                                                                        | 7.6                            | 76                    | 56              | 20                  | 60-65            | Passed.                        |
| (II)                                                                                                                       | 8                              | 50                    | 40              | 18                  | 60-65            | Do.                            |
| (VI)                                                                                                                       | 7.5                            | 45                    | 35              | 15                  | 60-65            | Do.                            |
| (LA) 60/40 blend of steam refined petroleum stock plus mineral lubricating oil (40 VI) containing additive mixture of (I). | 48.8                           | 409                   | 100             | 347                 | 45               | Failed.                        |
| (IB) Bright stock plus mineral lubricating oil (40 VI) containing additive mixture of (II).                                | 38.2                           | 277                   | 83              | 410                 | 40               | Do.                            |
| (IC) Same as I but lead sulfonate substituted for lead naphthenate in equal amount.                                        | 510                            |                       |                 |                     | 25               | Do.                            |
| (ID) Same as I but dibenzyl disulfide used for sulfurized sperm oil in equal amounts.                                      | 19                             |                       |                 | 820                 | 55               | Do.                            |

Compositions of the present invention can be used as extreme pressure lubricants for various heavy duty equipments operating under severe and adverse conditions of temperature and pressure.

I claim as my invention:

1. An improved gear oil composition consisting essentially of a mixture of two mineral oil fractions of: (1) 55-85% of a 90-140 VI Bright Stock having an aromatic content of at least 5% and (2) 45-15% of a mineral lubricating oil having a viscosity of 100-600 SUS at 100° F., viscosity index of at least 90 and 2-10% sulfur-containing aromatics of thiophenolic and benzo-thiophene structure and having incorporated therein from about 1% to about 10% each of lead naphthenate and sulfurized sperm oil.

2. An improved gear oil composition consisting essentially of a mixture of two mineral oil fractions of: (1) 55-85% of a 90-140 VI Bright Stock having an aromatic content of 5-70% and (2) 45-15% of a mineral lubricating oil having a viscosity of 100-600 SUS at 100° F., viscosity index of at least 90 and 2-10% sulfur-

containing aromatics of thiophenolic and benzothiophene structure and having incorporated therein from about 1% to about 10% each of lead naphthenate and sulfurized sperm oil.

5 3. The composition of claim 2 containing from about 0.1% to 5% each of polyisobutylene and 4,4-methylene-(2,6-ditert-butylphenol).

References Cited by the Examiner

UNITED STATES PATENTS

|    |           |         |                  |       |          |   |
|----|-----------|---------|------------------|-------|----------|---|
| 10 | 2,136,391 | 11/1938 | Miller           | ----- | 252-37.2 | X |
|    | 2,160,293 | 5/1939  | Shoemaker et al. | ----- | 252-45   |   |
|    | 2,607,732 | 8/1952  | Duchon et al.    | ----- | 252-37.2 |   |
|    | 2,704,745 | 3/1955  | Kopp et al.      | ----- | 252-37.2 |   |
| 15 | 2,816,867 | 12/1957 | Moore et al.     | ----- | 208-19   | X |
|    | 2,932,615 | 4/1960  | Jordan et al.    | ----- | 252-45   | X |
| 20 | 3,018,248 | 1/1962  | Foehr            | ----- | 252-37.2 |   |

DANIEL E. WYMAN, Primary Examiner.

CARL F. DEES, Assistant Examiner.